

March 23, 1954

T. W. GLYNN

2,673,142

ELECTRIC HEATING ELEMENT

Filed April 15, 1949

FIG. 1.



FIG. 2.



INVENTOR.  
THEODORE W. GLYNN

BY *Theodore W. Glynn*

ATTORNEYS

## UNITED STATES PATENT OFFICE

2,673,142

## ELECTRIC HEATING ELEMENT

Theodore W. Glynn, Kingsport, Tenn., assignor  
to Blue Ridge Glass Corporation, Kingsport,  
Tenn., a corporation of New York

Application April 15, 1949, Serial No. 87,754

4 Claims. (Cl. 41—42)

1

Heating elements made by the deposition of an electrically conducting grid on ceramic plates have the defect that the grid (generally of aluminum, silver, etc.) is subject to injury, thereby impairing the efficiency of the element and, furthermore, the grids unless protected by a second and non-conducting plate are liable to be short-circuited or grounded.

My invention has for its object a construction in which these objections are overcome, and to a method of applying and protecting the grid by which such improved heating elements may be more cheaply produced and for these ends consists in the feature hereinafter described and claimed.

Referring to the accompanying drawings in which similar parts are designated by similar marks of reference,

Figure 1 is a fragmental front view of a plate embodying my invention.

Figure 2 is a section on line 2—2 thereof.

The plate A may be of tempered glass coated with the selected conducting material B, say, aluminum, by a Schoop gun. Upon this uniform coating is impressed a design desired for the grid by placing over the coated plate a silk screen and applying thereto a medium having the characteristics set forth below. The medium passing through the silk screen imprints on the conducting coating the design of the grid. The plate with the medium thereon is then dried and baked at a temperature sufficient to harden and set the compound. The plate is then subjected to the action of a solvent capable of dissolving the conducting coating with which it may come in contact, but inert as to the baked medium. Thus, the deposited metallic coating is locally removed from the plate to leave the selected design for the grid thereon, all parts of the grid being covered by the hard and set medium C.

The medium to be used should have the following properties:

(a) Suitable viscosity and workability so that silk screen application is possible.

(b) After air drying or baking must be capable of protecting the aluminum coating from attack by the etching agent. The baking temperature should be as low as possible from the cost standpoint and cannot exceed the destraining temperature of the glass.

(c) Must adhere firmly to the aluminum so it is not removed in the washing operation that follows the etching process.

(d) Since it is to be left in place on the heater plate, it must be capable of enduring the operat-

2

ing temperature of the plate indefinitely without deterioration, discoloration, or oxidation, or change in electrical insulating properties.

(e) Must be odorless at the operating temperature of the plate.

(f) Must be an electrical insulator.

(g) Must be sufficiently elastic so that it will not crack or peel off of the plate under repeated cycles of heating and cooling.

10 (h) Must have sufficient abrasion resistance so that it is not scraped or knocked off the plate in ordinary handling operations before it is finally installed in the heating device.

(i) Must offer permanent protection to the 15 aluminum against the attack of acids, alkalies and corrosive fumes which might be encountered in its final service as a heating device.

I find that these properties are found in the mixture of:

|                         | Parts |
|-------------------------|-------|
| Silicone #996 varnish   | 860   |
| Ground titanium dioxide | 890   |
| Ground silica           | 29    |
| Lamp black              | 21    |

25 In this mixture the silicone varnish above referred to is one produced by the Dow-Corning Company and is a well-known article of commerce. It is used as the vehicle for the other ingredients and is selected for that purpose because of its heat-resisting properties. The titanium dioxide and silica are fillers and serve to stiffen the varnish to fit it for the silk screen process. Neither detracts from the insulating properties of the baked compound. The lamp black serves to give color to the design and to thus render inspection easier. It also increases the radiation from the exposed surface of the grid and should not be used where it is desired to suppress radiation from that side.

30 The plate with the design indicated thereon by the medium should then be baked or cured at a temperature of 250° C. for five minutes. The baking or curing temperature and time above given are subject to variation.

45 It is only necessary that the medium is set sufficiently to withstand the action of the solution to be subsequently applied, the final curing being effected when the plate is put in use as a heater. Likewise they are affected by the grade used. If silicone #803 is used instead of #996 the medium will air dry in about 16 hours and be ready for the solvent.

50 The solvent for the metallic coating is one fitted to dissolve the latter at points to which

it has access and inert as to the baked medium. With an aluminum coating and the compound of the medium before given, I find that a 30% solution of sodium hydroxide heated to about 60-80° C. is useful but an acid solution such as 5 diluted hydro-chloric acid may be used.

It will be found that in a plate prepared as above the bars of the grid will be sharply defined on the metal background, thus facilitating inspection.

It will be further found that the baked medium adheres closely to the metal on which it is deposited, forming a non-conducting and hard coating, thus protecting the metal and preventing short-circuit and grounding on accidental contacts. 15

What I claim is:

1. The hereinafter described method of making a heating element which comprises coating the surface of a ceramic plate with a metallic conducting coating, printing on such coating through a silk screen a selected design in a medium comprising a silicone varnish and a filler of non-conducting inorganic compounds of good 20 heat stability, baking the plate with the design thereon and removing the exposed portions of the metallic coating by a solvent inert to the printing medium. 25

2. The hereinafter described method of making a heating element which comprises coating the surface of a ceramic plate with a metallic conducting coating, printing on such coating through a silk screen a selected design in a medium comprising a silicone varnish and a filler of non-conducting inorganic compounds of good heat stability, and lamp black, baking the plate with the design thereon, and removing the exposed portions of the metallic coating by a solvent inert to the printing medium. 30

3. The hereinafter described method of mak-

ing a heating element which comprises coating the surface of a ceramic plate with a metallic conducting coating, printing on such coating through a silk screen a selected design in a medium comprising a silicone varnish and a filler of non-conducting inorganic compounds of good heat stability, drying the plate with the design thereon and removing the exposed portions of the metallic coating by a solvent inert to the printing medium. 10

4. The hereinafter described method of making a heating element which comprises coating the surface of a ceramic plate with a metallic conducting coating, printing on such coating through a silk screen a selected design in a medium comprising a silicone varnish and a filler of non-conducting inorganic compounds of good heat stability, drying the plate with the design thereon sufficiently to resist the solvent subsequently applied, removing exposed portions of the metallic coating by a solvent inert to the printing medium and thereafter drying and curing said medium under the heating effect of the electric current admitted to the metallic coating. 15

THEODORE W. GLYNN.

References Cited in the file of this patent

UNITED STATES PATENTS

| Number    | Name    | Date         |
|-----------|---------|--------------|
| 648,518   | Ochs    | May 1, 1900  |
| 2,022,827 | Ruben   | Dec. 3, 1935 |
| 2,081,894 | Meyer   | May 25, 1937 |
| 2,460,795 | Warrick | Feb. 1, 1949 |

FOREIGN PATENTS

| Number  | Country       | Date          |
|---------|---------------|---------------|
| 101,011 | Australia     | May 20, 1937  |
| 342,300 | Great Britain | Jan. 28, 1931 |
| 461,275 | Great Britain | Feb. 15, 1937 |